

# UNITED STATES PATENT OFFICE.

WILSON H. STRICKLER, OF COLUMBUS, OHIO.

## HEAT-RESISTING VULCANIZED FABRIC.

1,048,912.

Specification of Letters Patent. Patented Dec. 31, 1912.

No Drawing.

Application filed December 14, 1911. Serial No. 665,790.

*To all whom it may concern:*

Be it known that I, WILSON H. STRICKLER, a citizen of the United States, residing at Columbus, in the county of Franklin and 5 State of Ohio, have invented a new and useful Improvement in Heat-Resisting Vulcanized Fabric, of which the following is a specification.

This invention relates to a heat resisting 10 fabric especially adapted for use in manufacturing automobile and motor cycle tires, in connection with theater curtains, screens, or other articles in which a flexible heat resisting fabric is desirable.

15 The invention consists of a pliable fabric saturated with a rubber solution in which is thoroughly incorporated a suitable aluminate and finely ground or pulverized asbestos, said solution being applied to either 20 one or both sides of the fabric. It will be understood however, that the said solution is not simply a coating for the fabric but is thoroughly incorporated into it under suitable pressure, and further subjected to 25 a high temperature, so that the fabric and the rubber solution with the aluminate and the asbestos become practically one article.

In order that the said invention may be more fully understood a brief description 30 of the manner in which it is prepared is hereby given.

The fabric which may be of duck, canvas or any other suitable fabric is treated either upon one or both sides by a solution of 35 liquid rubber, to which has been added equal amounts of commercial aluminate, a mica preparation, and pulverized asbestos.

The term "aluminate" is a trade name employed to designate a certain mica preparation which I have found by careful experiments to be superior for the purpose intended than any other mica preparation I have been able to obtain. This term designates the finest ground mica put out and 45 is also known as commercial silicate of alumina, the word "aluminate" designating as before stated the product of a particular company.

The rubber solution is obtained by reducing the rubber to small pieces and then applying a suitable solvent, such as benzole or bisulfid of carbon, the former being preferred.

50 The combined mixture has a consistency about equal to that of cream and after the same has been applied to the fabric the

latter is passed between rolls so that the solution is thoroughly incorporated with the fibers of the fabric. I have found that where a rubber solution alone is employed 60 a tacky quality is given to the fabric. This fabric, however, lacks a heat resisting quality which I desire to obtain in combination with the tackiness above mentioned. The addition of the aluminate produces the desired heat resisting quality but deprives the completed article of a tacky quality. The addition of the asbestos restores this latter quality without in any way impairing the ability to resist heat imparted by the aluminate. 70

After passing through the pressing rolls the material is then dried after which it is given a second application, either to one or both sides, but in this second application 75 the amount of asbestos is reduced to one-third instead of one-half. The fabric is then subjected to a heat of about 275 degrees F. for about thirty minutes which cures or vulcanizes it, it is then ready for 80 use. The solution above mentioned may be applied to a clean fabric, or to a fabric which had previously been treated with rubber, or it can be applied to a sheet of rubber, which would replace the textile fabric. 85

The advantage gained by charging a textile base with a rubber solution carrying powdered mica and powdered asbestos consists in the fact that when these materials are brought into close combination with the fabric and are incorporated into the meshes and fiber of the fabric, they impart to the fabric after being thus incorporated their own distinctive qualities of heat resistance, making the fiber heat resistant when thus treated. The advantage of employing both the mica preparation and the asbestos has been fully pointed out and also the fact that the advantages claimed cannot be secured by the use of one of these substances only. 95

100 What I claim is:

1. A pliable sheet having rubber, pulverized asbestos, and finely ground mica, incorporated therein.

2. As a new article of manufacture, a pliable fabric having incorporated therewith a solution of rubber to which has been added a finely ground preparation of mica and pulverized asbestos. 105

3. A heat resisting fabric consisting of a textile base, and a rubber solution incorporated in said base, said solution having 110

incorporated therein a suitable mica preparation and pulverized asbestos.

4. A heat resisting fabric consisting of a textile base, and a rubber solution incorporated in said base and vulcanized thereto, said solution being treated with a finely ground mica preparation and pulverized asbestos prior to application of the solution to said base.

10 5. As a new article of manufacture a base

of textile fabric, a rubber solution having comminuted asbestos and a finely ground mica preparation incorporated therein, said rubber solution being pressed into the meshes of said fabric and thoroughly incorporated 15 with the fibers of said fabric.

WILSON H. STRICKLER.

Witnesses:

H. B. SNYDER,  
THOS. J. MURPHY.